

Feb. 3, 1970

O. R. BERGMANN ET AL

3,493,353

METAL COMPOSITES WITH LOW-MELT CONTENT BONDS

Original Filed Oct. 23, 1965

2 Sheets-Sheet 1

FIG. 1



INVENTORS

Oswald R. Bergmann  
George R. Cowan  
Arnold H. Holtzman

BY

*John O. Lehman*  
ATTORNEY

Feb. 3, 1970

O. R. BERGMANN ET AL

3,493,353

METAL COMPOSITES WITH LOW-MELT CONTENT BONDS

Original Filed Oct. 23, 1965

2 Sheets-Sheet 2

FIG. 3.

FIG. 3A.

FIG. 3B.



$\theta = 14.2^\circ$   
 $D = 2000 \text{ m/sec}$   
 $T = 1 \mu$



$\theta = 12.1^\circ$   
 $D = 2500 \text{ m/sec}$   
 $T = 3.1 \mu$



$\theta = 13.35^\circ$   
 $D = 3600 \text{ m/sec}$   
 $T = 9.2 \mu$

$\theta$  = PLATE IMPACT ANGLE  
 $D$  = COLLISION VELOCITY  
 $T$  = EQUIVALENT MELT THICKNESS  
 $M$  = MELT

FIG. 2.



DIRECTION OF DETONATION

BY

INVENTORS

OSWALD R. BERGMANN  
GEORGE R. COWAN  
ARNOLD H. HOLTZMAN

  
ATTORNEY

3,493,353

## METAL COMPOSITES WITH LOW-MELT CONTENT BONDS

Oswald R. Bergmann, Woodcrest, Cherry Hill Township, George R. Cowan, Woodbury, and Arnold H. Holtzman, North Cherry Hill Township, N.J., assignors to E. I. du Pont de Nemours and Company, Wilmington, Del., a corporation of Delaware

Original application Oct. 23, 1965, Ser. No. 503,261, now Patent No. 3,397,444. Divided and this application Jan. 19, 1968, Ser. No. 725,549

Int. Cl. B21d 39/00; B23p 3/00

U.S. Cl. 29—191

6 Claims

## ABSTRACT OF THE DISCLOSURE

Improved multilayered composites wherein two metallic layers of different composition are bonded together over at least 90% of their interface by a substantially diffusionless metallurgical bond and wherein said interface is substantially straight or in the form of waves of substantially uniform wave length and amplitude, and any solidified melt present at the interface is in localized regions spaced between areas of metal-to-metal metallurgical bonding, the solidified melt having an equivalent melt thickness of less than 1 micron.

This is a division of application Ser. No. 503,261, filed Oct. 23, 1965.

This invention relates to an improved process for cladding metals by means of explosives, and to improved clad products obtained thereby.

U.S. Patent 3,137,937 and copending, co-assigned U.S. patent application Ser. No. 217,776, now U.S. 3,233,312 describe a process for producing metallurgically bonded clad products by means of explosives. According to the process described, the metal layers to be metallurgically bonded together to form the clad product are positioned substantially parallel to one another and spaced apart a distance of at least 0.001 inch, and a layer of detonating explosive on the outside surface of at least one of the metal layers is initiated so that detonation is propagated parallel to the surfaces of the metal layers. The metal layer adjacent the explosive is propelled toward the other metal layer, collides with it, and is bonded thereto metallurgically. An essential condition of the described process is that the detonation velocity of the explosive be less than 120% of the velocity of sound in that metal in the system having the highest sonic velocity. The minimum detonation velocity set forth is about 1200 meters per second, this velocity being about the lowest at which commonly available explosives are found to propagate detonation reliably.

The above-cited patent and application show by way of detailed working examples the use of explosives having detonation velocities ranging from 3900 to 5000 meters per second. Such explosives in combination with the other process parameters outlined, afford strong continuously and metallurgically bonded (as opposed to mechanically bonded) clad products wherein the bond is substantially diffusionless and there are present regions, substantially homogeneous in composition, of alloy of the bonded metals. This alloy, which is solidified melt, is present either as a continuous layer between the bonded metals, or as a plurality of periodically spaced islands or regions separated by direct metal-to-metal metallurgical bonding. In the case of the continuous-layer type of bond, the general contour of the interface is substantially straight or irregularly curved, while in the case of the type of bond having alloy in periodically spaced regions, the interface between the bonded metals usually has a wavy contour.

Another explosion-bonding process is described in Belgian Patent 633,913. The process of the Belgian patent involves initially disposing the metal layers to be bonded at an angle to one another, positioning a layer of explosive adjacent the outer surface of at least one of the layers, and then detonating the explosive to drive the layers together.

It has now been found that under a certain specific narrow range of conditions within both of the aforementioned general processes, but preferably within the scope of the aforementioned explosion-bonding process described in U.S. Patent 3,137,937, there are obtained products having a unique combination of excellent strength, ductility, and freedom from solidification defects.

- 10 15 The process of this invention is an improvement in the process for metallurgically bonding layers of metals by propelling the layers together with an explosive, said improvement comprising effecting collision with respect to each of said metal layers at a velocity of about from 1400 to 2500 meters per second and below 120% of the sonic velocity of the metal in the system having the highest sonic velocity, the surfaces to be bonded of said layers being disposed at an angle of less than 10° to each other prior to detonation of said explosive.
- 20 25 The collision velocity is the velocity with which the line or region of collision travels along the metal layers to be bonded.

The unique and preferred products of this invention are multi-layered composites comprising at least two, and preferably two or three, metallic layers bonded together, adjacent layers in said composite being of different composition and metallurgically bonded over at least 90% of the interface therebetween, as-bonded, by a substantially diffusionless bond, said composite exhibiting ordered plastic deformation in a direction substantially parallel to said interface localized in the metal bonding each side thereof, any solidified melt present at said interface being present in localized regions between said layers and spaced between areas of metal-to-metal metallurgical bonding at said interface, said solidified melt having an equivalent melt thickness of less than one micron. As illustrated in the examples, the products of this invention have improved ductility reflected in a percent elongation of the composites, determined in accordance with ASTM Designation E8, preferably of at least 85% of the least ductile layer before bonding. Although products of this invention may contain regions of the alloy characteristic of explosion-bonded products generally, in all cases the amount of alloy is substantially less than that obtained heretofore and in some cases may not be observable at a magnification of 250×.

In accordance with this invention it has been found that as the collision velocity is decreased a critical velocity occurs below which the bonds change markedly even though all process variables except collision velocity are held constant. In addition, the effect of process variables differs significantly depending on whether the collision velocity is above or below the critical value. Although the critical velocity varies somewhat with the metals being clad, it is below about 2500 m./sec., and usually between 2300 to 2500 m./sec.

In the collision velocity region above the critical, the amount of solidified melt associated with the bond zone increases with collision velocity at any given impact angle (i.e., angle between metal layers on collision); also, when the interface is wavy, the wave amplitude is controlled by impact angle, increasing greatly with said angle. On the other hand, in the velocity region below the critical, there is little or no melt observable at 250× associated with the bond zone regardless of the impact angle, and the wave amplitude for a given metal system is significantly smaller

than that produced at the same impact angle at a collision velocity above the critical. Thus, operating in the below-critical region permits the obtaining of consistently low-melt products over a broad range of impact angles, i.e., a broad range of initial stand-off distances or initial angles between layers. Also, with a wavy interface, smaller-amplitude waves are obtained in a given system according to the present process. Extremely large wave amplitudes are undesirable when one or more layers of the clad composite are thin since the surface contour of the composite may be affected. Below 1400 m./sec., except with abnormally high explosive loading and/or stand-off distances, the products are not as strong as those obtained by the present process.

In the clad products formed by the present process, there is strong metallurgical bonding of the metal layers, substantially all of the bond being of the direct metal-to-metal type, that is, greater than 90% of the interfacial area between the metals being bonded is bonded by metal-to-metal bonding. Depending on the conditions used in the preparation of the clad product, e.g., the specific collision velocity and impact angle employed, the interface between the metallic layers can be in the form of a substantially straight line or in the form of a wave having a preferably uniform amplitude and wave length. Under most conditions, the wavy bond is formed. Any solidified melt which is present at the interface is present in isolated regions of such size that when the melt therein is converted into an equivalent continuous layer of uniform thickness along the entire interface, said layer is less than about ten microns, and usually less than one micron, thick. Stated differently, the total volume of melt divided by the area of the bonded interfaces is less than 10 microns, and preferably less than 1 micron. This "equivalent melt thickness" can be conveniently measured by taking a section through a sample parallel to the direction of detonation during bonding, measuring the total area of the melt in the section, and dividing such area by the length of the bonded interface. Clad products made by the present process and having at the interface an amount of melt which, when converted into an equivalent layer of uniform thickness along the entire interface, giving a layer less than one micron thick are preferred and unique products of this invention having particularly outstanding resistance to mechanical stresses. Such clad products having the wavy type of bond interface are preferred in many situations because of their normally higher strength.

In addition to providing an improved freedom from solidification defects, the present process also affords improved product workability, such as formability. Also, the ductility is relatively insensitive to changes in impact angle. Ductility of product is highly desirable in clad composites which are to be worked into various shapes.

Ordered plastic deformation of the metal bonding the interface between metal layers, as used herein with respect to the products of this invention, refers to regular gross plastic deformation in a general direction substantially perpendicular to the collision front occurring during the preparation of the products, i.e., in the direction of the collision, and generally parallel to and localized near the interface. The deformation follows the contour of the interface, e.g., in the case of wavy interfaces it follows the general contour of the waves, and is either precisely parallel to the interface or at some small acute angle thereto, e.g., 10-20°. As shown by the arrows in FIGURE 2, the aforementioned deformation is in a general direction away from a point or line in the composite. Stated differently, the arrows show plastic deformation in which the metal flow has been in the general direction of the detonation or collision during the bonding process, that is, deformation in the general direction away from the point or line of initiation of the explosive used in the bonding process. The plastic deformation is concentrated in the region adjacent the interface usually to a depth on either side thereof of less than about 25% of the thick-

ness of the thinner layer bonded at said interface, the depth of deformation in the case of a wavy interface being measured from a plane passing midway between the crests and troughs of the wave and normally being less than about 3 times the wave amplitude on either side of said plane.

Although as illustrated in the figures, the products are usually viewed in cross-section parallel to the direction of detonation, and, hence, any of the aforementioned melt appears as two-dimensional pockets, in reality any regions of solidified melt are elongated zones running parallel to the detonation front. The aforementioned melt, if observable, has a composition between that of the two layers between which it is disposed and the composition thereof is substantially homogeneous throughout each such region. The products are substantially diffusionless throughout in the as-bonded condition; that is, in the as-bonded condition the interface and adjacent areas, including the predominant metal-to-metal bonded regions as well as the alloy regions, if any, exhibit no gradient composition characteristic of diffusion-bonded products. Preferably, in the as-bonded condition they show no diffusion across any interface when measured with an electron probe and sectioning techniques having a limit of resolution of 0.2 micron. Especially preferred products are also characterized by a shear strength, measured parallel to the interface and substantially perpendicular to any waves therein, of at least about that of the parent metals before cladding. Any interfacial waves usually have an amplitude of about from 5 microns to 0.5 inch and normally no larger than about 50% of the thickness of the thinner layer bonded at the interface, and are substantially uniform in size throughout the composite. Such uniformity, which is a characteristic of the aforementioned preferred embodiment employing a layup having layers to be bonded in substantially parallel alignment, leads to particularly good uniformity of mechanical properties.

For a more complete understanding of the invention, reference is now made to the attached drawings wherein:

FIGURE 1 is a cross-sectional view of an assembly which can be used to practice the present invention;

FIGURE 2 is a photomicrograph (magnification of 76X) of a novel product of this invention showing the unique structure of the bond zone; and

FIGURES 3, 3A, and 3B are photomicrographs of clad products made at three different collision velocities.

In FIGURE 1, metal backer plate 1 and metal cladding plate 2 are parallel to one another and spaced apart so as to provide a stand-off 3. The stand-off spacing 3 can be conveniently maintained by metal ribbons 4 such as those described in U.S. Patent 3,205,574, the ribbons being positioned at the plate corners. A layer of a granular explosive 5 having a detonation velocity of about from 1400 to 2500 meters per second, held in container 6, e.g., made of cardboard, is adjacent the surface of metal layer 2 opposite the surface thereof facing metal layer 1. Explosive layer 5 extends beyond the parallel plate assembly and over metal strip 2a of the same composition and thickness as cladding plate 2. The metal strip and extension of the explosive layer are not critical to the process but provide added assurance that good bonding is achieved at the edge of the plates nearest the explosive initiation point. Explosive layer 5 is initiated by electric blasting cap 7 having lead wires 8 leading to a source of electricity. Upon initiation of explosive layer 5, plate 2 is propelled against plate 1 and collides progressively therewith as the detonation progresses through layer 5, the collision velocity being equal to the detonation velocity of explosive layer 5.

The photomicrographs shown in FIGURES 2, 3, 3A, and 3B are obtained on explosion-clad products described in the examples which follow, and the figures are described more fully therein.

In the improved cladding process of this invention, the metal layers collide at a collision velocity which is in

the region below the critical velocity described above, i.e., below about 2500 meters per second. Of two metal layers to be bonded, one may be propelled against the other, stationary, layer or both layers may be propelled toward each other to cause collision. Of three metal layers to be bonded, one metal layer may be propelled toward a second metal layer, which in turn is driven toward a third layer; or two outside layers can be propelled simultaneously toward an inside stationary layer. In like manner, with more than three layers, one or both outside layers can be propelled to cause collision and bonding. The metal layer or layers are propelled by the detonation of a layer of explosive or by another metal layer which is in turn propelled by detonation of a layer of explosive. The layers to be bonded can be arrayed initially parallel to, and spaced apart from, each other, or at some angle to one another. In either arrangement, the controlling parameters are so chosen that the collision velocity is about from 1400 to 2500 meters per second.

The collision velocity, as has been mentioned above, is the velocity with which the collision region travels along the metal layers to be bonded. More precisely, for two colliding layers 1 and 2, there are two collision velocities,  $V_{C1}$  and  $V_{C2}$ , denoting the velocities of the collision region relative to metal layers 1 and 2, respectively, that is, the velocities with which each of the two layers moves into the collision region or, stated differently, the velocities with which points on the inner surface of each of the layers approach the collision region. In most cases described herein the two velocities are the same or substantially the same; hence, there is little difference whether the velocities are considered as one or not. However, unless otherwise indicated, collision velocities of all layers being bonded must be within the indicated values.

In the preferred case of metal layers arrayed substantially parallel to one another, as in U.S. Patent 3,137,937 cited above, the layer of explosive is initiated so that detonation is propagated substantially parallel to the surfaces of the metal layers. If there is a layer of explosive adjacent only one of the metal layers, or if an explosive layer of the same detonation velocity is adjacent both metal layers and the explosive layers are initiated simultaneously at corresponding points or lines thereon, the collision velocities relative to both metal layers are equal to each other, and equal to the detonation velocity of the explosive. Thus, this embodiment of the present process employs explosives detonating at a velocity below about 2500 meters per second.

The explosion cladding of metal layers arrayed initially at an angle to one another is described in detail in Belgian Patent 633,913. Usually this angle should be less than  $10^\circ$  and preferably less than  $5^\circ$ . As explained therein, the parameters which affect the collision velocities differ depending on the manner of initiation of the explosive layer(s). When a layer of explosive on the external surface of one or of both metal layers is initiated simultaneously over its entire surface the collision velocities of the metal layers are functions of the initial angle  $\delta$  between the layers and their velocities  $V_{P1}$  and/or  $V_{P2}$ , the vector sum of which,  $V_P$ , is the velocity with which the metal layers are propelled toward one another. These relationships are:

$$(1) \quad V_{C1} = V_P / \tan \delta$$

$$(2) \quad V_{C2} = V_P / \sin \delta$$

Thus, for this arrangement the present process requires that the initial angle between the metal layers and the explosive loading (which affects the velocities of the propelled layer(s)) must be adjusted to provide a  $V_{C1}$  and  $V_{C2}$  of less than about 2500 meters per second.

The above-mentioned Belgian patent also teaches that when a layer of explosive on the external surface of one or both metal layers is initiated at a point or along a line the collision velocities of the metal layers are func-

tions of the initial angle  $\delta$  between the metal layers; the angles  $\gamma_1$  and/or  $\gamma_2$  by which the metal layer(s) are deflected by the detonation pressure; the angle  $\lambda$  which is the angle between the initial line of intersection of the planes of the metal plates and any line on the plates along which detonation is propagating; and the detonation velocity  $D$  of the explosive. Thus, in addition to the initial angle and the explosive loading (on which  $\gamma_1$  and  $\gamma_2$  depend), the method or location of the point or line of initiation and the detonation velocity of the explosive must be adjusted to provide a  $V_{C1}$  and  $V_{C2}$  of less than about 2500 meters per second. Relations for calculating  $V_{C1}$  and  $V_{C2}$  in these situations are (1), (m), (n), and (p) of the cited Belgian patent. Where a single layer of explosive is used:

$$\frac{V_{C1}}{D} = \frac{\sin \text{antitan} \left( \frac{[1 - \tan \gamma_1/2 \tan \delta \sin \lambda] \sin \gamma_1 \sin \lambda \cos \lambda}{\sin \gamma_1 + \cos \gamma_1 \tan \delta \sin \lambda - [1 - \tan \gamma_1/2 \tan \delta \sin \lambda] \sin \gamma_1 \cos^2 \lambda} \right)}{\cos \lambda}$$

$$\frac{V_{C2}}{D} = \frac{\sin \text{antitan} \left( \frac{\sin \lambda \cos \lambda}{\cos \delta [1 + \cot \gamma_1 \tan \delta \sin \lambda - \cos^2 \lambda]} \right)}{\cos \lambda}$$

Where explosive layers are positioned adjacent the external surface of both plates:

$$\frac{V_{C1}}{D} = \frac{\sin \text{antitan} \left( \frac{(1 - \tan \gamma_1/2 \tan \delta_1 \sin \lambda) \sin \gamma_1 \sin \lambda \cos \lambda}{\sin \gamma_1 + \cos \gamma_1 \tan \delta_1 \sin \lambda - (1 - \tan \gamma_1/2 \tan \delta_1 \sin \lambda) \sin \gamma_1 \cos^2 \lambda} \right)}{\cos \lambda}$$

$$\frac{V_{C2}}{D} = \frac{\sin \text{antitan} \left( \frac{(1 - \tan \gamma_2/2 \tan \delta_2 \sin \lambda) \sin \gamma_2 \sin \lambda \cos \lambda}{\sin \gamma_2 + \cos \gamma_2 \tan \delta_2 \sin \lambda - (1 - \tan \gamma_2/2 \tan \delta_2 \sin \lambda) \sin \gamma_2 \cos^2 \lambda} \right)}{\cos \lambda}$$

Deflection angles  $\gamma_1$  and  $\gamma_2$  can be measured in the same manner as plate velocities. One such method for measuring the velocity of an explosively propelled metal plate involves the use of electrical contact pins as is described by D. Bancroft, et al., Journal of Applied Physics, 27, (3), 291 (1956). An optical method is described by W. A. Allen and C. L. McCrary in Review of Scientific Instruments, 24 (2), 165 (1953) and by W. A. Allen, Journal of Applied Physics 24, (9), 1180 (1953); and a method involving use of flash X-radiographs is described by A. S. Balchan, ibid. 34, (2), 241 (1963). Also:

$$V_{P1} = 2D \sin \gamma_1/2 \quad (\text{or } V_{P2} = 2D \sin \gamma_2/2)$$

The angles  $\delta_1$  and  $\delta_2$  are solutions to the equations:

$$\begin{aligned} 55 \quad \delta_1 + \delta_2 &= \delta \\ \cos \delta (1 + \cos \gamma_1 \tan \delta_1 \sin \lambda - \cos^2 \lambda) \\ &= \cos \delta_2 (1 + \cot \gamma_2 \tan \delta_2 \sin \lambda - \cos^2 \lambda) \end{aligned}$$

The examples which follow show that when a collision velocity of about from 1400 to 2500 meters per second is employed in the explosion cladding technique, the geometry and composition of the bond zone in the clad product formed are less sensitive to changes in other process conditions, assuring that a desired bond zone character is achieved over a wider range of process conditions, e.g., metal layer velocity and impact angle (angle between layers at the collision region), as contrasted, e.g., with operating at higher than about 2500 meters per second. In particular, operation in the velocity region of this invention yields a low-melt bond zone and higher product ductility over a wide range of conditions, thus assuring product integrity under diverse conditions encountered in manufacture and processing. For optimum properties, reliability and reproducibility, collision velocities of 1900 to 2300 meters per second are preferred.

For any explosion cladding system, the occurrence of strong metallurgical bonding over a large proportion of the interface, is dependent not only on meeting the collision velocity requirement described above but also on the achieving of a certain minimum angle between metal layers on impact. For a given cladding system, operation in the collision velocity range of this invention appears to require a somewhat larger minimum impact angle than does operation in the above-2500-meters-per-second region. The larger impact angle can be produced by a larger initial stand-off or angle between layers or by use of a larger explosive load. Although the minimum impact angle varies from metal to metal, being about 4° for cladding systems containing nickel layers and 7° for titanium layers, generally it is in the range of 4° to 10°. In any case, an angle of 10° is usually adequate, the precise minimum being established by varying the stand-off, initial angle, or load. By way of example, for preferred systems involving layers consisting essentially of titanium or nickel (i.e., the indicated metals alone or alloys thereof with minor amounts of alloying elements) the impact angle is preferably about from 7° to 20° and 4° to 18°, respectively.

Standoff, loading, and initial angle can be varied as indicated within the broad teachings of U.S. Patent 3,137,937, Belgian Patent 633,913, and U.S. Serial No. 217,776 which are incorporated herein by reference; however, each of these interrelated variables are adjusted to optimize results with each particular system. In general, with the preferred technique employing layers in substantially parallel arrangement, point or line initiation and explosive on one or both sides of the layup, loading weights of about 0.2 to 3 times the driven or cladding layer weight are used, while standoffs of about from 0.3 to 0.7 of the cladding layer thickness are employed. Also, in general, explosive loading increases with the mass per unit area and standoff of the driven layer and usually is such that the driven layer has a velocity at collision of at least about 130 meters per second.

The explosive compositions useful in the present process vary widely and the selection of a particular composition will be made on the basis of such factors as the metal layer arrangement employed, ease of handling, economics, etc. In the preferred parallel cladding technique according to this invention, explosive compositions which detonate at velocities below about 2500 meters per second are employed. Typical of such compositions are nitro-  
guanidine in low bulk densities, self-supporting explosive sheets such as the fibrous felt-like compositions described in U.S. Patent 3,102,833, e.g., PETN and RDX sheets, and a number of permissible explosives such as some of those listed in the U.S. Bureau of Mines Information Circular 8087 (1962). When the angle cladding technique is employed, explosives having higher detonation velocities can be used, since the required collision velocity can be achieved with explosives of any higher detonation velocity by increasing initial angle (up to 10°) and/or explosive load.

The improved explosion cladding process of this invention is applicable to a wide variety of metals including, for example, aluminum, iron, titanium, columbium, chromium, tantalum, cobalt, nickel, vanadium, zirconium, silver, platinum, copper, gold, as well as alloys of a major portion, e.g., 50% by weight or more, of one or more of the aforementioned metals with minor amounts of alloying elements. Metals have a specific gravity of at least 2, and preferably from 4 to 17, particularly copper, nickel, iron, silver, titanium, zirconium, tantalum, and alloys of these metals are preferred. The alloys usually contain up to 50%, and preferably up to 30%, of alloying elements. In tantalum, titanium, and zirconium clads, usually the amount of alloying elements, is minor, e.g., less than 5%. Preferably, the difference in specific gravity between the metal layers being bonded is no greater than 9. Of course, for practical

purposes, the layers should be sufficiently ductile (e.g., per cent elongation of greater than 5%) so that they do not crack or fracture during the bonding process. In general, if a relatively brittle layer is to be bonded to a more ductile layer, explosive is positioned adjacent the more ductile layer and the more brittle layer is used as the backer. While the present process is employed to advantage in a number of metal systems, it affords particularly improved products in the case of metal systems which form brittle intermetallic phases, e.g., titanium-steel, zirconium-steel, tantalum-steel, and titanium-aluminum.

The technique employed to initiate the explosive layer(s), support the cladding assembly, prepare the metal surfaces, and otherwise effect the bonding process are described in the aforementioned patents, the disclosures of which are incorporated herein by reference. A particular effective means of maintaining the stand-off distance in the parallel technique is that shown in FIGURE 1, and described in detail in U.S. Patent 3,205,574. The manner of positioning of the assembly is not critical, e.g., a plate assembly can be positioned with the plate farthest from the explosive resting on the ground or on a support material on or in the ground. In some instances, it is convenient to position the assembly so that the plates are standing on their edges.

The process of this invention can be used to produce mill products, i.e., plates, sheets, strips, rods, bars, tubing, etc., comprised of at least two metallic layers of different composition bonded together over a large portion of the interface between the layers, e.g., over at least 90% of the interface, to form a composite system. The layers of different composition can be two layers of different substantially pure metals; two layers of different alloys (of the same or different metals); one layer of a substantially pure metal and a second layer of an alloy (of the same or a different metal than the first layer). Also, the product can be a composite of two or more layers bonded to a layer of substantially homogeneous composition; or of two or more multilayered composites bonded together. "Mill product" denotes here a product having a minimum significant dimension of three inches, e.g., a three-inch-long strip, rod, bar, or tube; and a plate or sheet having a length and width of at least three inches.

The following examples serve to illustrate specific embodiments of the present invention. However, they will be understood to be illustrative only and not as limiting the invention in any manner.

In all cases the metal surfaces are prepared by abrading with a disc sander and degreasing with alcohol.

The collision velocity given is the approximate detonation velocity of the explosive as measured from framing-camera sequences using a reflected grid-displacement technique, as are the plate velocity and plate impact angle. Such a technique is described by W. A. Allen and C. L. McCrary in *Review of Scientific Instruments*, vol. 24, pp. 165-171 (1953). The equivalent melt thickness is the total area of isolated pockets or regions of melt at the interface, in an illustrative cross-section parallel to the direction of detonation, divided by the length of the interface.

#### Example 1

A nickel plate is clad explosively to a steel plate employing the general arrangement depicted in FIGURE 1. The backer plate 1 is a 7 x 9 inch Grade 1008 steel plate  $\frac{1}{2}$  inch thick, and the cladding plate 2 is a 7 x 9 inch Grade A nickel plate  $\frac{1}{8}$  inch thick. Grade 1008 steel is a low-carbon or mild steel (about 0.08% carbon). The extension strip is a 1 x 7 inch strip of Grade A nickel  $\frac{1}{8}$  inch thick. The layer of explosives is a 70/30 nitro-  
guanidine/corn meal mixture in a loading of 15.4 grams per square inch. The collision (detonation) velocity is 2000 meters per second. The stand-off distance between plates is 156 mils. On detonation of the explosive, the plate impact angle is about 7°.

After detonation of the explosive, a specimen is cut out of the resulting well-bonded composite for metallographic examination of the bond zone. The interface is wavy and greater than 90% metallurgically bonded, and the equivalent melt thickness is less than  $1\mu$ . The product shows plastic deformation in the metal adjacent the interface in the direction of detonation.

If the procedure above is repeated using a silver plate of like size instead of the nickel above as the cladding layer, substantially similar results are obtained.

#### Example 2

The procedure described in Example 1 is used to explosively clad titanium ( $\frac{1}{8}$  inch) onto Grade 1008 steel ( $\frac{1}{2}$  inch). Grade 35-A titanium is used for the cladding

5 10 15

moving cladding plate. The conditions employed and results are summarized in Table I.

In all examples, bonding is effected over greater than 90% of the interface between plates.

The general direction of plastic metal flow near the bond zone in the clad products made according to the process of this invention is consistently away from the point or line at which the explosive has been initiated, or, in other terms, away from the center of curvature of a wave front emanating from the initiation point. This is seen in FIGURE 2, which is a photomicrograph ( $76\times$  magnification) made from the nickel-steel clad product of Example 7b. The direction of plastic flow is indicated by the arrows.

TABLE I.—NICKEL-STEEL CLADS

| Example No. | Collision Velocity (m./sec.) | Stand-Off (mils) | Plate Velocity (m./sec.) | Plate Impact Angle (degrees) | Bond Zone Characteristics |                       |                     |                                     |
|-------------|------------------------------|------------------|--------------------------|------------------------------|---------------------------|-----------------------|---------------------|-------------------------------------|
|             |                              |                  |                          |                              | Type                      | Wave Length ( $\mu$ ) | Amplitude ( $\mu$ ) | Equivalent Melt Thickness ( $\mu$ ) |
| 3.....      | a.....                       | 1,650            | 45                       | 215                          | 7.4 Straight and wavy ..  | 112                   | 10                  | <1                                  |
|             | b.....                       | 2,000            | 45                       | 250                          | 7.0 Wavy ..               | 103                   | 11                  | <1                                  |
|             | c.....                       | 2,500            | 45                       | 270                          | 6.6 do ..                 | 236                   | 39                  | 1.6                                 |
|             | d.....                       | 3,600            | 45                       | 410                          | 6.5 do ..                 | 254                   | 38                  | 5.1                                 |
| 4.....      | a.....                       | 2,000            | 85                       | 310                          | 8.7 do ..                 | 318                   | 41                  | <1                                  |
|             | b.....                       | 2,500            | 85                       | 337                          | 8.2 do ..                 | 425                   | 76                  | 3.9                                 |
|             | c.....                       | 3,600            | 85                       | 510                          | 8.25 do ..                | 590                   | 96                  | 9.8                                 |
| 5.....      | a.....                       | 1,650            | 156                      | 325                          | 11.2 do ..                | 520                   | 52                  | <1                                  |
|             | b.....                       | 2,000            | 156                      | 372                          | 10.5 do ..                | 567                   | 88                  | <1                                  |
|             | c.....                       | 2,500            | 156                      | 407                          | 9.7 do ..                 | 671                   | 121                 | 6.0                                 |
|             | d.....                       | 3,600            | 156                      | 625                          | 9.95 do ..                | 739                   | 146                 | 28.8                                |
| 6.....      | a.....                       | 2,000            | 250                      | 420                          | 11.8 do ..                | 790                   | 132                 | <1                                  |
|             | b.....                       | 2,500            | 250                      | 462                          | 10.8 do ..                | 895                   | 171                 | 9.0                                 |
|             | c.....                       | 3,600            | 250                      | 700                          | 11.2 do ..                | 965                   | 162                 | 24.0                                |
| 7.....      | a.....                       | 1,650            | 415                      | 425                          | 14.8 do ..                | 1,018                 | 169                 | <1                                  |
|             | b.....                       | 2,000            | 415                      | 460                          | 13.0 do ..                | 623                   | 97                  | <1                                  |
|             | c.....                       | 3,600            | 415                      | 775                          | 12.5 do ..                | 1,333                 | 284                 | 59.2                                |

plate and extension strip. The explosive loading is the same, the collision velocity is again 2000 meters per second, the stand-off distance between plates is 250 mils and the impact angle is about  $11\text{--}12^\circ$ . The composite is well-bonded over greater than 90% of its interface, and has a wavy interface. The equivalent melt thickness is less than  $1\mu$ , and the product shows plastic deformation adjacent the interface in the direction of detonation, primarily in the area within  $\frac{1}{32}$  inch from the interface on each side.

In all of the following examples, the detonation velocity can be decreased by increasing the amount of corn meal in the nitroguanidine/corn meal mixture, and increased (to velocities in the range below 3000 meters per second) by decreasing or eliminating the corn meal. For obtaining detonation velocities above 3000 meters per second, the explosive compositions described in U.S. Patent 3,102,833 can be used, the disclosure of that patent being incorporated herein by reference. As in the preceding examples, the explosive loading is such that the ratio of the weight of the mixture to the weight of the cladding plate is in the range of 0.2-3, the precise amount of explosive used being determined by adjusting the loading to give the indicated impact angle.

#### Examples 3-7

In these examples the procedure described in Example 1 is used to explosively clad a nickel plate to a steel plate. The stand-off distance between plates varies from example to example.

In each example, three or four experiments are described, each employing an explosive layer having a different detonation velocity than the others. Since the plates are initially parallel to one another, the collision velocity is equal to the detonation velocity of the explosive. The collision velocity and other fundamental process variables, i.e., cladding plate velocity and plate angle at impact, which prevail under the conditions of each experiment, are determined from framing-camera sequences of the

#### 10 15

moving cladding plate. The conditions employed and results are summarized in Table I.

In all examples, bonding is effected over greater than 90% of the interface between plates.

The general direction of plastic metal flow near the bond zone in the clad products made according to the process of this invention is consistently away from the point or line at which the explosive has been initiated, or, in other terms, away from the center of curvature of a wave front emanating from the initiation point. This is seen in FIGURE 2, which is a photomicrograph ( $76\times$  magnification) made from the nickel-steel clad product of Example 7b. The direction of plastic flow is indicated by the arrows.

#### Example 8

The procedure of Example 1 is repeated except that the explosive detonates at 1650 meters per second and the stand-off distance between plates is 700 mils. The plate velocity is 475 meters per second and the plate impact angle  $16.5^\circ$ . The composite is bonded over greater than 90% of the interface. The interface in this case is straight, and there is no detectable solidified melt in the bond zone 40 45 although there is deformation adjacent the interface in the direction of detonation. A sample cut from the clad is cold-rolled to 97% reduction in thickness with no sign of debonding.

#### Examples 9-13

The general procedure described in the preceding example is used to explosively clad titanium ( $\frac{1}{8}$  inch) onto Grade 1008 steel ( $\frac{1}{2}$  inch). Grade 35-A titanium is used. The conditions and results are reported in Table II. In all examples except Example 13b, bonding is achieved over greater than 90% of the interface. The ductility of the clad composites is measured in terms of percent elongation of 2-inch gauge length specimens obtained in a tensile test (ASTM Designation E8). The elongation 55 60 values given in the table are an average of three tensile tests for each clad composite. All tensile specimens are taken parallel to the direction of detonation.

As is seen from Table II, the ductility of clads made at 2000 meters per second collision velocities is greater than that of clads made at collision velocities above 2500 meters per second, especially as larger stand-offs are used. It is significant that the ductility values for the 2000-meters-per-second clads are rather constant over a wide range of stand-offs, while those for the higher-velocity clads decrease as stand-off increases. Thus, operating under the conditions of the present process, i.e., at collision velocities below about 2500 meters per second, permits uniformly desirable product properties to be obtained over wider ranges of operating conditions. The table also shows that wave amplitude and melt are

significantly reduced at low collision velocities within the scope of this invention.

appear in the bond zone, and at 3600 meters per second the melted areas are considerably larger in size.

TABLE II.—TITANIUM-STEEL CLADS

| Example No. | Collision Velocity (m./sec.) | Stand-Off (mils) | Plate Velocity (m./sec.) | Plate Impact Angle (degrees) | Type | Bond Zone Characteristics   |                     |     | Equivalent Melt Thickness ( $\mu$ ) | Tensile Test Elongation (percent) |
|-------------|------------------------------|------------------|--------------------------|------------------------------|------|-----------------------------|---------------------|-----|-------------------------------------|-----------------------------------|
|             |                              |                  |                          |                              |      | Wave Length ( $\mu$ )       | Amplitude ( $\mu$ ) |     |                                     |                                   |
| 9           | a.....                       | 2,000            | 45                       | 320                          | 9.9  | Wavy.....                   | 103                 | 8   | <1                                  | 32                                |
|             | b.....                       | 2,500            | 45                       | 400                          | 9.7  | do.....                     | 254                 | 19  | 1.2                                 | 32                                |
|             | c.....                       | 3,600            | 45                       | 580                          | 9.3  | Melted layer and waves..... | 250                 | 23  | 14.0                                | -----                             |
| 10          | a.....                       | 2,000            | 85                       | 420                          | 12.2 | Wavy.....                   | 215                 | 17  | <1                                  | 34                                |
|             | b.....                       | 2,500            | 85                       | 465                          | 11.0 | do.....                     | 482                 | 47  | 3.0                                 | 29                                |
|             | c.....                       | 3,600            | 85                       | 710                          | 11.3 | do.....                     | 468                 | 59  | 11.6                                | 28                                |
| 11          | a.....                       | 2,000            | 156                      | 495                          | 14.2 | do.....                     | 373                 | 31  | <1                                  | 31                                |
|             | b.....                       | 2,500            | 156                      | 520                          | 12.1 | do.....                     | 768                 | 89  | 3.1                                 | 29                                |
|             | c.....                       | 3,600            | 156                      | 845                          | 13.4 | do.....                     | 868                 | 122 | 9.2                                 | -----                             |
| 12          | a.....                       | 2,000            | 250                      | 530                          | 15.2 | do.....                     | 610                 | 53  | <1                                  | 32                                |
|             | b.....                       | 2,500            | 250                      | 565                          | 13.0 | do.....                     | 1,009               | 130 | 8.2                                 | 29                                |
|             | c.....                       | 3,600            | 250                      | 945                          | 15.0 | do.....                     | 1,228               | 189 | 18.5                                | -----                             |
| 13          | a.....                       | 2,000            | 415                      | 560                          | 15.5 | do.....                     | 1,013               | 96  | <1                                  | 32                                |
|             | b*.....                      | 2,500            | 415                      | 600                          | 14.0 | do.....                     | 1,300               | 167 | 3.6                                 | 27                                |
|             | c.....                       | 3,600            | 415                      | 1,040                        | 16.5 | do.....                     | 1,380               | 230 | 21.8                                | 23                                |

\* 80 % bonded.

The shear strength of the titanium-to-steel clad product made in Example 11a is determined both parallel and transverse to the direction of detonation. An average shear strength of  $50,000 \pm 2000$  p.s.i. is obtained for each direction. Shearing occurs in the steel backer rather than in the bond zone, however; therefore, the true shear strength of the bond zone is higher than the measured strength. In contrast to this, a titanium-to-steel clad made

25

### Examples 14-22

The procedure described in the preceding examples is used to prepare nine different clad composites. The conditions and results are shown in Table III. In all cases, bonding is achieved over more than 90% of the interface, and there is plastic deformation primarily in the area within 25% of the cladded layer thickness from the interface on each side.

TABLE III

| Example No.     | Cladder Metal (Thickness in inches)                                                                                                                                                                                                                                                                                                                       | Backer Metal (Thickness in inches) | Stand-Off (mils) | Collision Velocity <sup>2</sup> (m./sec.) | Bond Zone Characteristics                          |                                                    |                            | Equivalent melt thickness ( $\mu$ ) |
|-----------------|-----------------------------------------------------------------------------------------------------------------------------------------------------------------------------------------------------------------------------------------------------------------------------------------------------------------------------------------------------------|------------------------------------|------------------|-------------------------------------------|----------------------------------------------------|----------------------------------------------------|----------------------------|-------------------------------------|
|                 |                                                                                                                                                                                                                                                                                                                                                           |                                    |                  |                                           | Type                                               | Wavy (762 $\mu$ wave length, 102 $\mu$ amplitude.) | Similar to those of Ex. 14 |                                     |
| 14              | Grade A Nickel (0.125)                                                                                                                                                                                                                                                                                                                                    | Copper (0.5)                       | 156              | 1,650                                     | Wavy (762 $\mu$ wave length, 102 $\mu$ amplitude.) | -----                                              | -----                      | <1                                  |
| 14a             | Repetition of Ex. 14 except that 2 layers of 0.125 inch nickel are clad onto the 0.5 inch copper layer simultaneously by positioning the explosive on the outside surfaces of both nickel layers and initiating both explosive layers simultaneously. The same explosive loading and stand-off used in Ex. 14 are used for each Ni-Cu pair in the system. | -----                              | -----            | -----                                     | -----                                              | -----                                              | -----                      | -----                               |
| 15 <sup>1</sup> | Tantalum (0.05)                                                                                                                                                                                                                                                                                                                                           | Grade 1008 Steel (0.5)             | 60               | 1,900                                     | Straight.....                                      | -----                                              | -----                      | <1                                  |
| 16              | 304L Stainless Steel (0.06)                                                                                                                                                                                                                                                                                                                               | 5083-0 Aluminum (0.75)             | 45               | 2,200                                     | do.....                                            | -----                                              | -----                      | <1                                  |
| 17              | 304L Stainless Steel (0.125)                                                                                                                                                                                                                                                                                                                              | do.....                            | 45               | 2,100                                     | do.....                                            | -----                                              | -----                      | ~5                                  |
| 18a             | 35-A Titanium (0.19)                                                                                                                                                                                                                                                                                                                                      | 304 Stainless Steel (0.75)         | 200              | 2,300                                     | Wavy.....                                          | -----                                              | -----                      | <1                                  |
| 18b             | do.....                                                                                                                                                                                                                                                                                                                                                   | do.....                            | 200              | 2,800                                     | do.....                                            | -----                                              | -----                      | >10                                 |
| 19              | Grade 11 Zirconium (0.125)                                                                                                                                                                                                                                                                                                                                | A212B FRQ <sup>3</sup> Steel (1.0) | 80               | 2,200                                     | do.....                                            | -----                                              | -----                      | <1                                  |
| 20              | do.....                                                                                                                                                                                                                                                                                                                                                   | 304L Stainless Steel (0.75)        | 175              | 2,200                                     | do.....                                            | -----                                              | -----                      | <10                                 |
| 21              | Grade 11 Zirconium (0.19)                                                                                                                                                                                                                                                                                                                                 | A212B FRQ Steel (1.0)              | 175              | 2,200                                     | do.....                                            | -----                                              | -----                      | <10                                 |
| 22              | Grade 11 Zirconium (0.375)                                                                                                                                                                                                                                                                                                                                | do.....                            | 300              | 2,300                                     | do.....                                            | -----                                              | -----                      | <10                                 |

<sup>1</sup>Clad composite from Example 15 is reduced by 98% of its thickness by cold-rolling, without failing.

<sup>2</sup>Detonation velocity measured by pin method, except in Example 14 (framing camera).

<sup>3</sup>A medium-carbon steel.

using a collision velocity of 2800 meters per second gives 50 an average shear strength of only about 40,000 p.s.i.

Bond integrity of the clad product is also determined from the ability of the product to withstand cold-rolling. The product made in Example 11a can be reduced to 66% of its thickness by cold-rolling in a direction normal to the direction of detonation without debonding. As a comparison, a titanium-steel clad product is made under the same conditions as used in Example 11a except that the explosive has a detonation velocity of approximately 3200 meters per second. The plate velocity is 790 m./sec. and plate impact angle 13.8°. The product is 100% bonded, the bond zone consisting of a wavy zone with pockets of melt. The wave length is 1017 $\mu$ , amplitude 139 $\mu$ , and the average thickness of the melt 16 $\mu$ . The product debonds completely after only a 35% reduction in thickness by cold-rolling.

FIGURES 3, 3A and 3B show the influence of collision velocity on the amount of melt produced in the titanium clads of Example 11, i.e., those made at a constant stand-off of 156 mils and nearly constant plate impact angle, but at three different collision velocities. As is seen from the photomicrographs of the figures, there is practically no melt in the bond zone at 2000 meters per second. At 2500 meters per second, melted pockets of increasing size

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660</p

is given in the above-cited Belgian Patent 633,913 (second part of relation *m*). According to this determination, the collision velocity is approximately 1460 meters per second.

The clad composite is found to be metallurgically bonded over more than 90% of the interface. The interface is in the form of waves having a wave length of 1250 microns and an amplitude of 99 microns. The equivalent melt thickness is less than one micron.

We claim:

1. A multilayered composite comprising two metallic layers of different composition bonded together over at least 90% of their interface by a substantially diffusionless, metal-to-metal metallurgical bond, and wherein

- (a) said interface is substantially straight or is in the form of waves of substantially uniform wave length and amplitude, and any solidified melt present at the interface is in localized regions between said layers and is spaced between areas of metal-to-metal metallurgical bonding, said solidified melt having an equivalent melt thickness of less than one micron, and
- (b) said layers exhibit ordered plastic deformation in a direction substantially parallel to said interface and localized in the metal bounding each side of said interface,

said composite having a percent elongation of at least 85% of the least ductile layer before bonding.

2. A product of claim 1 wherein said interface is in the form of waves of uniform wave length and amplitude.

3. A product of claim 1 wherein the metals of said layers comprise a metals system which forms brittle intermetallic phases.

4. A product of claim 2 wherein said metal layers are selected from the group consisting of copper, nickel, iron, silver, titanium, zirconium, tantalum, and alloys thereof.

5. A product of claim 4 wherein one of said layers is low-carbon steel.

6. A product of claim 4 wherein said metal layers consist of titanium or zirconium bonded to steel.

10

15

20

25

#### References Cited

#### UNITED STATES PATENTS

|           |        |                    |        |
|-----------|--------|--------------------|--------|
| 3,233,312 | 2/1966 | Cowan et al. ----- | 29—194 |
| 3,397,045 | 8/1968 | Winter -----       | 29—191 |

L. DEWAYNE RUTLEDGE, Primary Examiner

G. K. WHITE, Assistant Examiner

U.S. Cl. X.R.

29—194, 196, 198, 199